

Patented Oct. 14, 1930

1,778,634

## UNITED STATES PATENT OFFICE

MAX HARTMANN, OF RIEHEN, NEAR BASEL, AND WILLI KLARER, OF BASEL, SWITZERLAND, ASSIGNORS TO THE FIRM SOCIETY OF CHEMICAL INDUSTRY IN BASLE, OF BASEL, SWITZERLAND

## TREATMENT OF METALS WITH ACID LIQUORS

No Drawing. Application filed June 4, 1929, Serial No. 368,426, and in Switzerland June 7, 1928.

The present invention relates to an improvement in the art of pickling iron, especially malleable iron, steel, iron alloys and articles therefrom, as wires, wire ropes, sheets, etc. It comprises the new pickling liquors, the process of making same, the application thereof, as well as the metal treated with the new pickling liquors.

This invention is based on the observation that quite generally the products soluble in dilute mineral acids which are obtained by condensing aldehydes, ketones and suitable acid chlorides, such as phosgene, with aromatic amino-compounds or aromatic nitro-compounds and subsequent reduction are remarkably suitable additions to acid liquids for treating metals. They are particularly suitable as additions to pickling baths, liquid soldering fluxes or the like, which serve for removing from metals impurities, such as rust, scale or the like.

These products comprise quite generally compounds containing at least two aryl nuclei which themselves contain an  $\text{NH}_2$ -group or a substituted  $\text{NH}_2$ -group and which are bound by a so-called central carbon atom. This central carbon atom itself may be bound with hydrogen, oxygen, alkyl or aryl residues.

Among these products or classes of products there may be mentioned diaminodiphenylmethane, diaminoditolylmethane, diaminodiphenylmethane or the corresponding symmetrical and unsymmetrical primary or secondary N-substitution products, for example 4:4'-tathamethyldiaminodiphenylmethane; further the corresponding products which may be obtained with acetaldehyde or acetone instead of with formaldehyde; as well as ketones, such as 4:4'-tetramethylaminobenzophenone, also the triaminotriphenylmethane or, quite generally, the leuco-compounds of the triarylmethane dyestuffs containing amino-groups, such as leuco-crystal violet or leuco malachite green, or the

corresponding quaternary ammonium bases of all these compounds. Particularly suitable are the products the salts of which correspond to the general formula



wherein  $\text{R}_1$ ,  $\text{R}_2$ ,  $\text{R}_3$ ,  $\text{R}_4$ ,  $\text{R}_5$ ,  $\text{R}_6$ =hydrogen, alkyl, aralkyl or aryl,  $\text{R}_7$ =hydrogen or alkyl, and  $\text{R}_8$ =hydrogen, alkyl or aryl, and wherein  $\text{z}$  and  $\text{y}$  means the same or different anions.

It has been found most unexpectedly that these compounds, when added even in very small proportions to acid liquid, prevent more or less completely the attack of metals by these liquids without, however, affecting the solvent action of the liquids for rust, oxide or the like. The advantages of such an addition are clear; there is saving of metal and acid, diminution of the formation of hydrogen and acid vapors accompanied by diminished brittleness due to the pickling, and increased protection for the worker who has to carry out the operation of pickling.

The above mentioned compounds may be used not only alone or in mixture with each other but also in combination with various substances, such as mineral salts, sulfite cellulose liquor, sulfonated oils, mono- and unsymmetrical di-acylated diamines and the corresponding ammonium bases, tar products or the like.

The following examples illustrate the invention, the parts being by weight:—

## Example 1

1000 parts of hydrochloric acid of 15 per cent. strength are mixed with 0.2 part of the hydrochloride of 4:4'-tetramethylaminodiphenylmethane or with 0.1 part of the hydrochloride of 4:4'- or 2:2'-tetramethylaminodiphenylmethane. The solution may

50

55

60

65

70

75

80

85

90

used at once as an agent for treating metals.

*Example 2*

1000 parts of hydrochloric acid of 15 per cent. strength are mixed with 0.1 part of the hydrochloride of 3:3'-diamino-4:4'-dimethyldiphenylmethane. The product may be used immediately as an agent for treating metals.

*Example 3*

1000 parts of hydrochloric acid of 15 per cent. strength are mixed with 0.1 part of the hydrochloride of 4:4'-tetramethyldiamino-diphenylmethane and 0.9 part of sulfite cellulose liquor. The solution can be used at once as a metal treating agent.

*Example 4*

Sheet iron is immersed until it has been completely pickled in a pickling liquor containing per 1000 parts of hydrochloric acid of 15 per cent. strength 0.2 part of the hydrochloride of 4:4'-tetramethyldiaminodiphenylmethane or with 0.1 part of the hydrochloride of 4:4'- or 2:2'-tetramethyldiaminodiphenylmethane. The pickling is finished in a short time without dissolution of noticeable quantities of the metal. The sheets are then removed and are ready for further treatment (tinning, zincing, varnishing, soldering or the like). If for any reason the iron is not immediately removed from the pickling liquor there is no appreciable further action of the acid and in consequence practically no dissolution of the metal, such as is known to occur in a pickling bath of the ordinary kind.

The same results are obtained with the corresponding tetraethyl-compounds.

In like manner a pickling bath consisting of sulfuric acid or mixtures of acids may be treated; instead of the compounds mentioned in the examples other compounds as disclosed in the introduction hereto may be used. The operation may be conducted cold or hot.

What we claim is:—

1. Pickling baths containing compounds soluble in dilute mineral acids and corresponding with the general formula



55 wherein  $R_1$ ,  $R_2$ ,  $R_3$ ,  $R_4$ =hydrogen, alkyl, aralkyl or aryl,  $R_5$ =hydrogen or alkyl, and  $R_6$ =hydrogen, alkyl or aralkyl.

2. Pickling baths containing compounds soluble in dilute mineral acids and corresponding with the general formula



65 wherein  $R_1$ ,  $R_2$ ,  $R_3$ ,  $R_4$ ,  $R_5$ ,  $R_6$ =hydrogen or alkyl.

3. Pickling baths containing compounds soluble in dilute mineral acids and corresponding with the general formula



70

wherein  $R_1$ ,  $R_2$ ,  $R_3$  and  $R_4$ =hydrogen or such alkyls which contain not more than two carbon atoms.

4. Pickling baths containing compounds soluble in dilute mineral acids and corresponding with the general formula



80

wherein  $R_1$ ,  $R_2$ ,  $R_3$  and  $R_4$ =hydrogen or such alkyls which contain not more than two carbon atoms, and wherein aryl stands for a benzene or naphthalene nucleus.

5. Pickling baths containing compounds soluble in dilute mineral acids and corresponding with the formula



85

In witness whereof we have hereunto signed our names this 24th day of May, 1929.

MAX HARTMANN.

WILLI KLARER.

95

100

105

116

113

123

123

130